

## UNITED STATES PATENT OFFICE

STUART A. FALCONER, OF ELIZABETH, AND LUDWIG J. CHRISTMANN, OF JERSEY CITY, NEW JERSEY, ASSIGNEES TO AMERICAN CYANAMID COMPANY, OF NEW YORK, N. Y., A CORPORATION OF MAINE

## METHOD AND AGENT FOR RECOVERY OF OXIDIZED ORES

No Drawing.

Application filed June 1, 1931. Serial No. 541,528.

The object of this invention is the separation of minerals, especially of oxide minerals, from ores containing the same by froth flotation.

Many reagents are known which are promoters for sulfide ores but not all sulfide reagents are effective in the flotation of so-called oxidized minerals. On the other hand, reagents for oxidized minerals will, in general assist in the flotation of sulfides.

By an oxide mineral we mean one composed of a heavy metal such as lead, zinc, copper, etc., in connection with elements or groups of elements other than sulfur.

It has been known that mercaptobenzothiazole possessed promoter properties for assisting in the flotation of oxide minerals but it is too insoluble as such and is best used in the form of its sodium or potassium salt. Although such salts are of some value in the flotation of oxidized ores, we have found that by dissolving mercaptobenzothiazole in a solution of sodium sulfide it is possible to obtain much better flotation results than when the sodium or potassium salt of mercaptobenzothiazole is used either alone or in conjunction with sodium sulfide or with the polysulfides  $\text{Na}_2\text{S}_2$ ,  $\text{Na}_2\text{S}_3$ ,  $\text{Na}_2\text{S}_4$  or  $\text{Na}_2\text{S}_5$ .

A series of tests was run on an ore from Africa. The ore contained a considerable amount of the copper as chrysocolla. The analysis of the sample was as follows:

|                         | Per cent |
|-------------------------|----------|
| Total copper            | 11.28    |
| Non-sulfide copper      | 10.48    |
| Iron                    | 4.80     |
| $\text{Al}_2\text{O}_3$ | 4.33     |
| Lead                    | Trace    |
| Zinc                    | Trace    |
| $\text{MgO}$            | 1.41     |
| $\text{Cl}_2$           | Trace    |
| Sulfur                  | 0.92     |
| Manganese               | 0.088    |
| Insoluble               | 65.70    |
| Gold                    | Trace    |
| Silver                  | Trace    |

The ore which consisted of minus  $\frac{1}{4}$  inch particles and fines was stage crushed by passing through a set of rolls to minus 10 mesh

ore and 600 cc. of water were ground in a steel laboratory rod mill for a period of 18 minutes.

A screen analysis showed:

| Mesh  | % Weight | 55 |
|-------|----------|----|
| + 65  | -----    |    |
| + 100 | 0.50     |    |
| + 150 | 2.00     |    |
| + 200 | 7.00     |    |
| + 250 | 3.50     |    |
| + 300 | 10.10    | 60 |
| - 300 | 76.90    |    |

The ground charge was transferred to a laboratory subaeration type of flotation machine and diluted to 22% solids. A total time of float of 18 min. was used but the reagents were added in stages.

When the sodium salt of mercaptobenzothiazole was used alone, very poor results were obtained. When sodium sulfide was used together with the sodium salt of mercaptobenzothiazole, the results were improved. The use of sodium poly sulfides in conjunction with sodium mercaptobenzothiazole gave about the same results as sodium sulfide. However, when mercaptobenzothiazole dissolved in sodium sulfide solution was used, greatly improved results were obtained, the increase in recovery of copper being as high as 10% over that obtained with the combination of the sodium salt of mercaptobenzothiazole and sodium sulfide.

The following table outlines, in general, the procedure followed, giving the time of the flotation treatment, the amounts of reagents used, and the intervals at which they were added.

| Reagent                              | Reagents added, pounds per ton of ore minutes |       |       |       |       |       |       |       |       |
|--------------------------------------|-----------------------------------------------|-------|-------|-------|-------|-------|-------|-------|-------|
|                                      | Start                                         | 2     | 4     | 6     | 8     | 10    | 12    | 14    | 16    |
| Sodium salt of mercaptobenzothiazole | 0.50                                          | 0.25  | 0.25  | 0.25  | 0.25  | 0.25  | 0.25  | 0.25  | 0.25  |
| Sulfidizing agent                    | 0.50                                          | 0.25  | 0.25  | 0.25  | 0.25  | 0.25  | 0.25  | 0.25  | 0.25  |
| Oleic acid                           | 0.046                                         | 0.023 | ----- | ----- | ----- | 0.046 | ----- | ----- | ----- |
| Pine oil                             | 0.021                                         | 0.021 | ----- | ----- | ----- | 0.021 | ----- | ----- | ----- |

When mercaptobenzothiazole dissolved in 100

sodium sulfide was used, the first addition was equivalent to one pound of combined reagent per ton and the additions at two minute intervals were equivalent to 0.5 pounds per ton.

The following table gives the comparative results obtained with the sodium salt of mercaptobenzothiazole and the various sulfidizing reagents:

| Products % Cu | Reagents: Pounds per ton |       |       |                                                      |                                   |                   |                                |                                | % Cu recovery                  |      |
|---------------|--------------------------|-------|-------|------------------------------------------------------|-----------------------------------|-------------------|--------------------------------|--------------------------------|--------------------------------|------|
|               | Heads                    | Conc. | Tails | Mercaptobenzothiazole dissolved in Na <sub>2</sub> S | Mercaptobenzothiazole sodium salt | Na <sub>2</sub> S | Na <sub>2</sub> S <sub>2</sub> | Na <sub>2</sub> S <sub>3</sub> | Na <sub>2</sub> S <sub>4</sub> |      |
|               |                          |       |       | 5.0                                                  | 2.5                               | 2.5               | 2.5                            | 2.5                            | 2.5                            |      |
| 15            | 11.00                    | 20.45 | 3.59  | 5.0                                                  | 2.5                               | 2.5               | 2.5                            | 2.5                            | 2.5                            | 81.7 |
|               | 11.00                    | 23.85 | 4.70  | -----                                                | 2.5                               | 2.5               | 2.5                            | 2.5                            | 2.5                            | 71.4 |
|               | 11.10                    | 24.80 | 4.11  | -----                                                | 2.5                               | 2.5               | 2.5                            | 2.5                            | 2.5                            | 75.6 |
| 20            | 11.10                    | 24.40 | 4.39  | -----                                                | 2.5                               | 2.5               | 2.5                            | 2.5                            | 2.5                            | 73.8 |
|               | 11.08                    | 24.10 | 4.72  | -----                                                | 2.5                               | 2.5               | 2.5                            | 2.5                            | 2.5                            | 71.4 |
|               | 11.12                    | 23.05 | 5.10  | -----                                                | 2.5                               | 2.5               | 2.5                            | 2.5                            | 2.5                            | 69.6 |

\*A 6% solution of the above reagent is prepared by dissolving three parts by weight of mercaptobenzothiazole in 100 parts of water containing three parts by weight of fused sodium sulfide.

From the table it is readily seen that the results obtained with mercaptobenzothiazole dissolved in sodium sulfide are by far the best by from 6.1% to 12.1% additional copper recovery.

On another sample of oxidized ore in which the copper mineral was largely malachite, an experiment was run under the same conditions as above and the following results were obtained.

| % Cu | Pounds per ton |       |       | % Cu recovered |      |
|------|----------------|-------|-------|----------------|------|
|      | Heads          | Conc. | Tails |                |      |
|      |                |       |       |                |      |
| 40   | 15.68          | 30.20 | 1.15  | 4.0            | 96.3 |
|      | 15.75          | 33.20 | 1.88  | 2.0            | 93.3 |

Here again better results are obtained when the mercaptobenzothiazole is dissolved in the sodium sulfide as the amount of copper recovered was increased by 3%, a very notable increase.

Instead of dissolving the mercaptobenzothiazole in sodium sulfide reagent, we may grind the two solids together. By this procedure a uniform product is obtained easily soluble directly in water.

The reaction which takes place between the ingredients may be represented as follows:



While we do not know with certainty the reasons for the effectiveness of our composition as a promoter of flotation we believe that the combination forms sodium hydrosulphide which acts as a sulfidizing agent and which at

the same time imparts only a low degree of alkalinity. This is of great advantage, in that it minimizes the tendency to form soluble compounds of the heavy metals with alkalis and thus render such metals more amenable to the flotation operation. Furthermore, our invention provides a most inexpensive and convenient means for solubilizing mercaptobenzothiazole and at the same time obtaining the available sodium hydrosulphide. Although we have described our invention setting forth a single embodiment thereof it is apparent that many variations in composition and in procedure may be made within the scope of our invention. For example, we may use different proportions of mercaptobenzothiazole and of sodium sulfide with good results. Instead of sodium sulfide other alkali metal sulfides, such as ammonium sulfide, potassium sulfide and the like may be used. Our invention is not limited to the treatment of copper ores but is applicable to the treatment of ores of other metals, such as lead, zinc and the like and particularly ores of oxidized character.

What we claim is:

1. In the flotation concentration of ores, the method which comprises adding to the flotation circuit as a promotor a mixture of mercaptobenzothiazole and an alkali metal sulfide.

2. In the flotation concentration of ores, the method which comprises adding to the flotation circuit as a promotor a mixture of mercaptobenzothiazole and sodium sulphide.

3. In the flotation concentration of ores, the method which comprises adding to the flotation circuit as a promotor, a mixture of sodium mercaptobenzothiazole and an alkali metal hydrosulphide.

4. In the flotation concentration of ores, the method which comprises adding to the flotation circuit as a promotor, a mixture of sodium mercaptobenzothiazole and sodium hydrosulphide.

5. A composition of matter comprising mercaptobenzothiazole and an alkali metal sulphide.

6. A composition of matter comprising mercaptobenzothiazole and sodium sulphide.

7. A composition of matter comprising sodium mercaptobenzothiazole and an alkali metal hydrosulphide.

8. A composition of matter comprising sodium mercaptobenzothiazole and sodium hydrosulphide.

In witness whereof, we have hereinto subscribed our names this 27th day of May, 1931.

STUART A. FALCONER.  
LUDWIG J. CHRISTMANN.